

3,850,949

PHOTORESITIVE MATERIAL FOR ELECTRO-PHOTOGRAPHY INCLUDING INDOLINE DERIVATIVES

Hisatake Ono, Syu Watarai, and Harumi Katsuyama, Asaka, Japan, assignors to Fuji Photo Film Co., Ltd., Kanagawa, Japan

No Drawing. Filed Oct. 6, 1971, Ser. No. 187,190  
Claims priority, application Japan, Oct. 6, 1970,  
45/87,788

Int. Cl. C07d 85/16

U.S. Cl. 260—307 F

4 Claims

ABSTRACT OF THE DISCLOSURE

An organic photoconductive material for electrophotography consisting essentially of indoline derivatives represented by the following general formula (A)

(A)



wherein R<sub>1</sub> is hydrogen atom, halogen atom, alkyl group having 1 to 4 carbon atoms, alkoxy group having 1 to 4 carbon atoms, alkoxy carbonyl group having alkyl group having 1 to 4 carbon atoms, nitro group, or alkylene chain having 1 to 3 carbon atoms, R<sub>2</sub> is hydrogen atom, hydroxyl group, alkoxy carbonyl group having alkyl group having 1 to 4 carbon atoms, cyan or phenyl group, R is substituted phenyl group (wherein substituted group is hydrogen atom, halogen atom, alkyl group having 1 to 4 carbon atoms, or alkoxy group having 1 to 4 carbon atoms), alkylene chain having 1 to 3 carbon atoms or phenylene group, m is an integer from 1 to 4.

This invention relates to an organic photoconductive material for electrophotography. As photoconductive materials applicable to electrophotography there are known inorganic substances such as selenium and zinc oxide, organic lower molecular compounds such as anthracene, chrysene and benzidine, and higher molecular compounds such as poly-N-vinylcarbazole, polyvinyl naphthalene and polyvinylanthracene.

This invention relates to an organic photoconductive material having a novel structure completely different from known materials, and provides a photosensitive material having as an essential component 2-substituted-methylene-indoline derivatives represented by the following general formula (A):



wherein R<sub>1</sub> is hydrogen atom, halogen atom, alkyl group having 1 to 4 carbon atoms, alkoxy group having 1 to 4 carbon atoms, alkoxy carbonyl group having alkyl group having 1 to 4 carbon atoms, nitro group, or methylene

chain having 1 to 3 carbon atoms, R<sub>2</sub> is hydrogen atom, hydroxyl group, alkoxy carbonyl group having alkyl group having 1 to 4 carbon atoms, cyan or phenyl group, R is substituted phenyl group (wherein substituted group is hydrogen atom, halogen atom, alkyl group having 1 to 4 carbon atoms or alkoxy group having 1 to 4 carbon atoms), methylene chain having 1 to 3 carbon atoms or phenylene group, m is an integer from 1 to 4.

The above formula (A) is represented by the following formulae (I) to (IV).

(I)



15

(II)



20

(III)



25

(IV)



30

35

40

45

50

55

60

65

70

75

80

85

90

95

100

105

110

115

120

125

130

135

140

145

150

155

160

165

170

175

180

185

190

195

200

205

210

215

220

225

228

230

235

240

245

250

255

260

265

268

270

275

280

285

290

295

300

305

310

315

320

325

330

335

340

345

350

355

360

365

370

375

380

385

390

395

400

405

410

415

420

425

430

435

440

445

450

455

460

465

470

475

480

485

490

495

500

505

510

515

520

525

530

535

540

545

550

555

560

565

570

575

580

585

590

595

600

605

608

610

615

620

625

630

635

640

645

650

655

660

665

670

675

680

685

690

695

700

705

708

710

715

720

725

730

735

740

745

750

755

760

765

770

775

780

785

790

795

800

805

808

810

815

820

825

830

835

840

845

850

855

860

865

870

875

880

885

890

895

900

905

910

915

920

925

930

935

940

945

950

955

960

965

970

975

980

985

990

995

1000

1005

1010

1015

1020

1025

1030

1035

1040

1045

1050

1055

1060

1065

1070

1075

1080

1085

1090

1095

1098

1099

1100

1105

1110

11

1,3-dipolar cyclo-addition to multiple bonds such as acetylene, nitrile, carbonyl, olefin and the like. Mechanism of these reactions is known as dipole ring formation reaction, and concerning it R. Huisgen wrote general considerations in *Angewandte Chemie*, 75, 604 (1963). Recently synthesis of polymers containing heterocycles utilizing the 1,3-dipolar cycloaddition reaction were reported, for instance, see Iwakura, Shiraishi et al. *Bulletin of the Chemical Society of Japan*, 38, 335 (1965); *ibid.*, 38, 513 (1965); and *Polymer Letters*, 4, 305 (1966) etc.

With reference to these reports, many addition products were obtained by reacting various 2-methyleneindolines with various hydroxamic acid halides in the presence of a base. It was proved that the structure of these addition products is a spiro (indoline-2,5'-isoxazoline) structure from the results of elemental analysis and measurements of infrared absorption spectrum, ultraviolet absorption spectrum, visible ray absorption spectrum, NMR spectrum, etc. For instance 1,3,3-trimethyl-2-methylene-5-chloroindoline and benzhydroxamic acid chloride were dissolved in ether. To the solution was added dropwise, 1N sodium hydroxide solution and the mixture was stirred at room temperature for 30 minutes. Then the ether layer was dried and concentrated, in reduced pressure and crystals were obtained.

Thus isolated compound was colorless, needle-like and had a melting point of 167 to 168° C. and had the following results of elemental analysis: carbon 69.49%, hydrogen 5.86%, nitrogen 8.36%. The results were in good agreement with theoretical value of 1,3,3-trimethyl-5-chloro-3'-phenyl-spiro (indoline-2,5'-isoxazoline)



carbon 69.59%, hydrogen 5.86%, nitrogen 8.57%. Meanwhile, the agreement was supported by the fact that the parent peak ( $M^+$ ) of mass spectrum was 326, and the compound had the absorption in infrared absorption spectrum at  $1560\text{ cm}^{-1}$  which agreed with  $\nu c=N$ , and had a maximum absorption in ultraviolet absorption spectrum at  $262\text{ m}\mu$  ( $\epsilon=2.58\times 10^4$ ). On the basis of these

absorptions it was concluded that the compound had an indoline type structure altered from the methylene-indoline type structure starting material. Moreover, in NMR spectrum (tetramethylsilane dissolved in deuterated chloroform solution, internal reference) the compound had peaks at  $\delta$  value (as p.p.m.) 1.25 (S, 3H), 1.34 (S, 3H), 2.61 (S, 3H), 3.03, 3.33, 3.38, 3.39 (AB type 2H,  $J=18.0$  c.p.s.) and ring protons (8H) were observed.

On the basis of above-mentioned data it is obvious that the compound of this invention has spiro (indoline-2,5'-isoxazoline) structure.

Meanwhile, a high polymer compound obtained by the reaction of 5,5'-methylenebis-(1,3,3-trimethyl-2-methylene-indoline) with dichloroglyoxime had a maximum absorption in ultraviolet absorption spectrum at  $262\text{ m}\mu$ , and in NMR spectrum the high molecular compound had peaks at  $\delta$  value 1.24 (S), 1.37 (S), 2.66 (S), 3.01, 3.34, 3.67 (Transition type to  $A_2$  type from AB type) and multiplet ring protons (8H). The intensity ratio of these peaks was 6:6:4:2:6, and infrared absorption spectrum also agreed nearly with spectrum of the above mentioned mono-spiro-compound. From these data it is obvious that the high molecular compound of this invention has a structure containing spiro-(indoline-2,5'-isoxazoline) as repetition unit.

In this invention, it was found that the many compounds which were prepared and which had structures which were confirmed as stated above are useful as organic photoconductive materials for electrophotography. These compounds are listed in Table 1 to Table 4.

The high molecular compounds of this invention are soluble in various organic solvents such as chloroform, tetrahydrofuran, N,N-dimethylformamide, N,N-dimethylacetamide, N-methyl-2-pyrrolidone and the like, and are so highly polymerized that they give a strong film by applying a solution of the polymer in a lower boiling solvent such as tetrahydrofuran to a metallic plate and drying, and their reduced viscosity value ( $\eta_{sp.}/c$ ) was about from 0.03 to 0.6.

TABLE 1



| Compound number | $R_1$                             | $R_3$          | M.P. (°C.)  | $\text{CHCl}_3$ | $\lambda_{\text{max.}}$ | $(M\mu)_1 (\epsilon)$ |
|-----------------|-----------------------------------|----------------|-------------|-----------------|-------------------------|-----------------------|
| 1               | —H                                | —H             | 118         | 260             | $(1.95\times 10^4)$     |                       |
| 2               | —Cl                               | —H             | 167-168     | 262             | $(2.58\times 10^4)$     |                       |
| 3               | —H                                | —Cl            | 170-171     | 268             | $(2.18\times 10^4)$     |                       |
| 4               | $\text{C}_2\text{H}_5\text{OCO}-$ | —H             | 123-124     | 304             | $(3.07\times 10^4)$     |                       |
| 5               | $-\text{NO}_2$                    | —Cl            | 184-185     | 265             | $(2.16\times 10^4)$     |                       |
| 6               | $-\text{NO}_2$                    | —H             | 210.5-211.5 | 260             | $(1.88\times 10^4)$     |                       |
| 7               | $\text{CH}_3\text{O}-$            | —H             | 155         | 259             | $(1.94\times 10^4)$     |                       |
| 8               | —H                                | $-\text{CH}_3$ | 140         | 260             | $(2.05\times 10^4)$     |                       |

TABLE 2



| Compound number | $R_1$                             | $R_4$                       | M.P. (°C.) | $\text{CHCl}_3$ | $\lambda_{\text{max.}}$ | $(M\mu)_1 (\epsilon)$ |
|-----------------|-----------------------------------|-----------------------------|------------|-----------------|-------------------------|-----------------------|
| 9               | —H                                | Direct bond of carbon atoms | 231        | 259             | $(3.06\times 10^4)$     |                       |
| 10              | —Cl                               | do                          | 154        | 262             | $(4.08\times 10^4)$     |                       |
| 11              | $\text{C}_2\text{H}_5\text{OCO}-$ | do                          | 242        | 305             | $(4.64\times 10^4)$     |                       |
| 12              | —H                                | $-\text{CH}_2-$             | 200        | 259             | $(3.30\times 10^4)$     |                       |
| 13              | —H                                | $(-\text{CH}_2-)_3$         | 185        | 259             | $(3.21\times 10^4)$     |                       |
| 14              | —H                                |                             | 273        | 299             | $(3.30\times 10^4)$     |                       |

TABLE 3



| Compound number | <i>n</i> | <i>m</i> | <i>R</i> <sub>2</sub>             | <i>R</i> <sub>3</sub> | M.P. (°C.) | $\lambda_{CHCl_3 \text{ max}}$ | ( $\epsilon$ )        |
|-----------------|----------|----------|-----------------------------------|-----------------------|------------|--------------------------------|-----------------------|
| 16              | 0        | 2        | -COOC <sub>2</sub> H <sub>5</sub> | -H                    | 210        | 265                            | (5.78 $\times 10^4$ ) |
| 17              | 1        | 1        | -H                                | -H                    | 196        | 264                            | (4.32 $\times 10^4$ ) |
| 18              | 1        | 1        | -H                                | P-Cl-                 | 250        | 274                            | (3.97 $\times 10^4$ ) |

TABLE 4



| Compound number | <i>n</i> | <i>m</i> | <i>R</i> <sub>2</sub>                          | <i>R</i> <sub>4</sub>         | Reaction time (hr.) | Yield, percent | M.P. (°C.) | $\eta_{sp./c.}$ , solvent |
|-----------------|----------|----------|------------------------------------------------|-------------------------------|---------------------|----------------|------------|---------------------------|
| 19              | 0        | 1        | -H                                             | Direct bond of carbon atoms.. | 1                   | 80             | 273-275    | 0.15 (THF).               |
| 20              | 1        | 1        | -H                                             | ----do----                    | 20/60               | 90             | >300       | 0.49 (THF).               |
| 21              | 1        | 1        | -H                                             | ----do----                    | 3                   | 90             | 230-240    | 0.11 (THF).               |
| 22              | 1        | 2        | -CO <sub>2</sub> C <sub>2</sub> H <sub>5</sub> | ----do----                    | 20/60               | 70             | 174-185    | 0.06 (THF).               |
| 23              | 1        | 1        | -H                                             |                               | 1                   | 90             | 300        | 0.27 (NMP).               |
| 24              | 0        | 1        | -H                                             |                               | 20/60               | (i)            | >300       | Impossible to measure.    |
| 25              | 1        | 1        | -H                                             |                               | 1                   | 80             | >300       | 0.15 (NMP).               |
| 26              | 0        | 3        | -CN                                            | Direct bond of carbon atoms.. | 1                   | 90             | >300       | 0.11 (THF).               |
| 27              | 2        | 2        | -OH                                            | ----do----                    | 1                   | 50             | 250-270    | 0.07 (THF).               |

<sup>1</sup> Quantitative.

For utilizing lower molecular compounds which were above-mentioned for use as materials for electrophotography, coatings as light-sensitive layer are made by dissolving the compounds in organic solvents with highly insulating coating-forming resinous binders, applying the solutions to comparatively electroconductive supports and drying, if desired. It is also possible to add plasticizers and sensitizers thereby to improve the characters of coatings and to increase greatly the sensitivity. In the case of high molecular compounds listed in Table 4, coatings for use as a light-sensitive layer are made by dissolving the high molecular compounds in organic solvents without highly insulating coating-forming resinous binder, applying the solution to comparatively electroconductive supports and drying, if desired. It is also possible to add plasticizers and sensitizers thereby to improve the characteristics of the coatings and to increase greatly the sensitivity.

As coating-forming resinous binders, styrene-butadiene copolymers, polystyrenes, chlorinated rubbers, polyvinyl chlorides, vinyl chloride/vinyl acetate copolymers, polyvinylidene chloride, nitrocelluloses, polyvinyl acetates, polyvinylacetals, polyvinyl ethers, silicon resins, methacrylic resins, acrylic resins, phenol resins, alkyd resins, urea/aldehyde resins, etc. may be used, and as electroconductive supports, metallic plates, electroconductive papers, electroconductive plastic films, etc. may be used, and as plasticizers chlorinated biphenyls, chlorinated paraffins, phosphate plasticizers, phthalate plasticizers, etc. may be used, and as sensitizers, conventional sensitizers such as tetracyanoethylene, tetracyanoquinodimethane,

chloranil, naphthoquinone, anthraquinone, Methylene Blue, Crystal Violet and Malachite Green, etc. may be used.

It is preferred to suitably combine these materials and apply them on an electroconductive support to provide a dried coat of 2 to 20 microns in thickness. When organo-photoconductive component is more than 25 percent of the total components of the coating, electrophotographically excellent characteristics are obtained.

The light-sensitive layer obtained by above-mentioned process is uniformly charged by corona discharge according to the conventional method of electrophotography, and after image-exposure is developed by cascade development, liquid development, etc. In the case of cascade development it may be fixed by weakly heating after development or by standing in solvent-vapor capable of dissolving the resin of toner.

This invention is further illustrated by the following examples. However, this invention shall not be limited to the following examples.

#### EXAMPLE 1

Half a gram of compound No. 1 in Table 1 and 20 ml. of 10% polystyrene solution in tetrahydrofuran were blended uniformly, the resulting solution was applied to an aluminum plate support to provide a dried coating of 0.5 micron in thickness.

After drying it was charged with positive electricity in a dark place, and a positive picture film was placed upon it, then they were exposed with a high-pressure

